

## UNITED STATES PATENT OFFICE

HANS T. CLARKE AND CARL J. MALM, OF ROCHESTER, NEW YORK, ASSIGNEES TO EASTMAN KODAK COMPANY, OF ROCHESTER, NEW YORK, A CORPORATION OF NEW YORK

## PROCESS OF MAKING CELLULOSE ESTERS OF CARBOXYLIC ACIDS

No Drawing.

Application filed March 28, 1927. Serial No. 179,177.

This invention relates to processes of making cellulose esters of carboxylic acids. One object of the invention is to provide a process of such general applicability that the cellulose esters of many different organic acids, even those of high molecular weight, may be prepared by means of it. Another object is to provide such a process in which organic acids containing the acidic groups for the esters may be used directly without the trouble and expense of preparing their anhydrides or chlorides. A further object is to provide such a process in which a high proportion of the acidic groups available for the cellulose ester is actually combined into the ester, without being wasted. Another object is to provide a cellulose-esterifying process in which, as a main initial ingredient, there is an anhydrid of an organic acid, which anhydrid does not contain a cellulose-esterifying group or hydrolyze to an acid containing such a group,—in other words, the anhydrid impels esterification without contributing any groups to the esters produced.

Another object of the invention is to provide a relatively simple process which will be rapid, economical and easily controlled. A still further object is to provide a process which will esterify, not only easily esterified cellulosic bodies, such as hydrocellulose and reverted cellulose, but can also and preferably utilize substantially undegraded cellulose, such as cotton, surgical cotton wool, tissue paper from cotton stock, and even sulfite wood pulp, thereby producing cellulose esters of higher quality. Another object is to provide such a process in which the ingredients form a liquid active esterifying bath at temperatures which do not substantially impair the cellulose or the cellulose esters. A still further object is to provide a process which, as it proceeds, produces a solvent that helps to keep the esterifying ingredients in proper solution. Other objects will hereinafter appear.

We have found that these objects may be attained, in general, by subjecting the cellulosic material to the coaction of an organic acid containing a cellulose-esterifying group and an organic acid anhydrid which impels

such esterification without itself supplying any cellulose-esterifying groups as disclosed in our copending application 179,176. By the term cellulose-esterifying groups, we refer to those which are capable of combining with the cellulose under the conditions of our process. The organic acids which we can employ for furnishing such groups can be selected from the group which consists of the unsubstituted aliphatic monocarboxylic acids including the cycloparaffinic, the aromatic monocarboxylic acids and the aralkyl monocarboxylic acids. Typical anhydrids which can be used in our process to impel esterification, without furnishing cellulose-esterifying groups, include the halogen or alkoxy substituted fatty acid anhydrids. Of these, the ones having less than ten carbon atoms are the most convenient to use. In fact, we prefer to use a chlorinated acetic anhydrid, the anhydrid of monochloracetic acid (hereinafter referred to for convenience as chloracetic anhydrid) being as advantageous as any other and less expensive.

The time of the process is shortened and the results are more advantageous when a catalyst is used. While we may employ any of the catalysts which have hitherto been used successfully in the production of cellulose acetate from acetic anhydrid, we prefer to utilize the milder ones, such as the perchlorates disclosed in the application of Carl J. Malm, Serial No. 137,385, filed September 23rd, 1926 for process of making cellulose esters of organic acids. Zinc chloride is satisfactory, but we prefer magnesium perchlorate. We can also use red phosphorus and chlorine,—see U. S. Patent No. 1,591,590, Webb and Malm, July 6th, 1926.

Our process is carried out at temperatures above the melting points of the ingredients of the esterifying bath, but below temperatures at which the cellulose, or the esters made from it, are degraded. Such degradation is indicated by brittleness of films prepared from the esters. It should be noted that when the ingredients of our baths are mixed together the mixture usually has a lower melting point than the melting points of the ingredients, taken alone. It should

further be noted that the halogen substituted fatty acid anhydrides, especially those containing less than ten carbon atoms, have a strong solvent action upon the acids which we employ, as stated above. For instance, chloracetic anhydrid has a good solvent action on such difficulty soluble materials as stearic acid. Moreover, the monochloracetic acid, which is formed from said anhydrid during the esterification is likewise a strong and satisfactory solvent of the acids. There is, therefore, no danger of premature precipitation of the ingredients as the reaction proceeds. While the general range of available temperatures is indicated above, we find it especially convenient to work between 50° C. and 80° C., according to the particular acids and halogenated fatty acids anhydrides employed. As will be seen by the examples hereinafter given, rapid esterification may be accomplished in a comparatively short time, without degradation of the product, at a temperature of 60° to 65° C., when acetic anhydrid and magnesium perchlorate are employed.

Our process can utilize cellulosic materials from any of the sources customarily used in the manufacture of esters, such as cotton fiber tissue paper, clean cotton, surgical cotton wool, and even sulfite wood pulp, (preferably bleached). These materials, especially the cotton materials, are undegraded when they enter our process and yield esters which are likewise substantially unimpaired or undegraded, as evidenced by the flexibility of films prepared from them. But our process is likewise applicable to cellulosic materials which have been chemically affected, such as so-called hydrocellulose, reverted cellulose, such as from the viscose or cuprammonium processes and lower cellulose nitrates, acetates, formates, or ethers still containing esterifiable hydroxyls.

We shall now give numerous examples of our process by way of illustration, but it will be understood that our invention is not limited to the details thus given, except as indicated in the appended claims. Taking one of the simplest cases, a bath is prepared by mixing 25 parts by weight of glacial acetic acid with 30 parts by weight of chloracetic anhydrid and 0.05 parts of magnesium perchlorate trihydrate. Into this, after the ingredients are well mixed, there is thoroughly incorporated 5 parts by weight of clean cotton. During the esterification this bath is kept between 60° to 65° C. The completion of acetylation is indicated by the disappearance of the cotton fibers, the reaction mass becoming homogeneous. This occurs comparatively rapidly,—say in about three hours. The completed ester is obtained from the bath by treatment which follows customary practice. For example, the bath may be poured, with stirring,

into cold methyl alcohol, or any other solvent of the fatty acid, which is not a solvent of the product. Precipitation in cold water is, therefore, possible with our process. Where the latter is employed, the organic acids in the solution may be obtained either by extraction with volatile organic solvents or by concentration, neutralization, evaporation and treatment of the salts thus obtained, as is well known to chemists skilled in the art. Where precipitation into an organic liquid takes place, the acids, especially the chloracetic acid, may be recovered by fractional distillation, under a partial vacuum, when necessary. Some of the chloracetic values may be alternatively recovered by conducting air through the reaction mass, while the latter is strongly agitated, and then conducting the air to a condensing chamber to remove chloracetic vapors from it, this air being warmed and then recirculated through the reaction mixture. Here again the operating temperature is kept low enough to avoid injuring the ester, preferably well under 130° C. See U. S. Letters Patent No. 1,494,816, Seel, May 20th, 1924, No. 1,560,620, Sulzer, November 10th, 1925, and No. 1,516,225, Webb, November 18th, 1924, for examples of similar recoveries.

For convenience we have arranged the following examples in tabular form:

| Name of the acid       | Solubilities of final products at room temperature |                           |                                         |                                          |                  |            |                         |               |          |            |            |
|------------------------|----------------------------------------------------|---------------------------|-----------------------------------------|------------------------------------------|------------------|------------|-------------------------|---------------|----------|------------|------------|
|                        | Parts of acid by weight                            | Parts of cotton by weight | Parts of chloracetic anhydrid by weight | Parts of magnesium perchlorate by weight | Time of reaction | In acetone | In carbon tetrachloride | In chloroform | In ether | In benzene | In ligroin |
| Acetic                 | 25                                                 | 5                         | 30                                      | 0.05                                     | 3                | —          | —                       | —             | —        | —          | —          |
| Propionic              | 25                                                 | 5                         | 30                                      | 0.05                                     | 3                | +          | —                       | +             | —        | —          | —          |
| n-butyric              | 10                                                 | 3                         | 20                                      | 0.05                                     | 4                | +          | +                       | +             | —        | +          | —          |
| Iso-butyric            | 15                                                 | 3                         | 25                                      | 0.05                                     | 4                | +          | +                       | +             | +        | +          | —          |
| n-valeric              | 15                                                 | 3                         | 25                                      | 0.05                                     | 4                | +          | +                       | +             | +        | +          | —          |
| Iso-valeric            | 15                                                 | 3                         | 25                                      | 0.05                                     | 4                | +          | +                       | +             | +        | +          | —          |
| n-caproic              | 20                                                 | 5                         | 60                                      | 0.05                                     | 4                | +          | +                       | +             | +        | +          | —          |
| n-heptylic             | 18                                                 | 4                         | 55                                      | 0.05                                     | 8                | +          | +                       | +             | +        | +          | —          |
| Caprylic               | 25                                                 | 5                         | 60                                      | 0.05                                     | 5                | +          | +                       | +             | +        | +          | —          |
| Pelargonic             | 25                                                 | 5                         | 60                                      | 0.05                                     | 5                | +          | +                       | +             | +        | +          | —          |
| Caprie                 | 25                                                 | 5                         | 60                                      | 0.05                                     | 5                | +          | +                       | +             | +        | +          | —          |
| Lauric                 | 20                                                 | 3                         | 20                                      | 0.05                                     | 4                | —          | —                       | —             | —        | —          | —          |
| Myristic               | 25                                                 | 4                         | 60                                      | 0.05                                     | 4                | —          | —                       | —             | —        | —          | —          |
| Palmitic               | 15                                                 | 2                         | 60                                      | 0.05                                     | 24               | —          | —                       | —             | —        | —          | —          |
| Stearic (comm.)        | 15                                                 | 2                         | 60                                      | 0.05                                     | 24               | —          | —                       | —             | —        | —          | —          |
| Crotonic               | 15                                                 | 5                         | 30                                      | 0.05                                     | 5                | +          | —                       | +             | —        | +          | —          |
| Cyclohexane-carboxylic | 10                                                 | 2                         | 15                                      | 0.02                                     | 3                | —          | —                       | —             | —        | —          | —          |
| Benzole                | 15                                                 | 3                         | 20                                      | 0.05                                     | 8                | —          | —                       | —             | —        | —          | —          |
| o-methoxy-benzoic      | 10                                                 | 2                         | 15                                      | 0.02                                     | 4                | —          | —                       | —             | —        | —          | —          |
| o-chloro-benzoic       | 10                                                 | 2                         | 15                                      | 0.02                                     | 5                | —          | —                       | —             | —        | —          | —          |
| Acetyl salicylic       | 20                                                 | 2                         | 20                                      | 0.05                                     | 10               | —          | —                       | —             | —        | —          | —          |
| Phenylacetic           | 15                                                 | 3                         | 20                                      | 0.05                                     | 7                | —          | —                       | —             | —        | —          | —          |
| Hydrocinnamic          | 15                                                 | 3                         | 30                                      | 0.05                                     | 3                | +          | +                       | +             | —        | —          | —          |
| Cinnamic               | 15                                                 | 3                         | 40                                      | 0.05                                     | 5                | —          | —                       | —             | —        | —          | —          |
| Stearic (comm.)        | 30                                                 | 4                         | 50                                      | 0.05                                     | 7                | +          | —                       | +             | —        | —          | —          |
| Acetic                 | 6                                                  | 4                         | 50                                      | 0.05                                     | 7                | +          | —                       | +             | —        | —          | —          |
| o-methoxy-benzoic      | 10                                                 | 2                         | 15                                      | 0.02                                     | 7                | +          | —                       | +             | —        | —          | —          |
| Acetic                 | 15                                                 | 2                         | 20                                      | 0.02†                                    | 3                | —          | —                       | +             | —        | —          | —          |
| Acetic                 | 10                                                 | 2                         | 20                                      | 0.05*                                    | 6                | —          | —                       | +             | —        | —          | —          |

† Trichloracetic anhydrid was used in place of the monochloracetic.  
\* Betabromopropionic anhydrid was used in place of the monochloracetic.

(a) Soluble in warm ligroin, insoluble at room temperature.

120

In all of the above examples the working temperature is kept between 60° and 65° C. In the six columns at the right, which indicate the solubilities, a minus sign indicates that the ester, which is produced, does not dissolve in the particular liquid in question, at least not to any readily detectable or useful extent. A plus sign indicates that it does have a useful solubility in such a solvent at room temperature. For example, the cellulose acetostearate produced in the fourth from the last example in the table is soluble in acetone and chloroform but insoluble in benzol. As will be evident from the third and fourth examples from the bottom of the table, we may obtain mixed esters by using mixtures of the acids in any desired proportions. The third from the last example gives cellulose aceto-orthomethoxybenzoate. In the case of the unsubstituted monocarboxylic aliphatic acids containing a double bond, the latter should preferably be situated in the alpha-beta position relatively to the carboxyl group. Thus crotonic and cinnamic acids act well.

Moreover, we may usefully have present chloracetic acid at the start of the reaction in addition to the amount of such acid formed during the reaction. For example, we may prepare a bath by mixing 300 parts by weight of chloracetic anhydrid, 100 parts by weight of chloracetic acid, 185 parts of stearic acid, 35 parts of acetic acid, and 0.5 parts of magnesium perchlorate. Into this is stirred 25 parts by weight of cellulose and the reaction mixture kept for about 8 hours at 60° to 65° C. A clear dope is thus obtained and the mixed cellulose ester is separated, and the other ingredients recovered, as indicated hereinabove. The mixed ester is soluble in acetone and insoluble in benzene. Analysis shows it to contain 40% of stearyl and palmityl groups and 22% of acetyl groups. Its acetone solutions can be formed into films which are colorless, transparent and of very high flexibility either with or without the addition of plasticifying substances, such as triphenyl phosphate.

In another example, we may mix 155 parts by weight of chloracetic anhydrid, 190 parts by weight of chloracetic acid, 92 parts of stearic acid, 20 parts of acetic acid, and 0.3 parts of magnesium perchlorate. 25 parts by weight of cellulose are treated in this mixture at 60° to 65° C. until a clear dope is formed, say for about 12 hours. The ester is separated and washed as hereinabove described. It is soluble both in acetone and benzene. Analysis shows it to contain 55% of palmityl and stearyl groups and 15% of acetyl groups.

Furthermore, our process operates satisfactorily when in place of the acid or acids which furnish the esterifying groups, there are substituted in whole or in part the cor-

responding acid anhydrids. In fact, such anhydrids are potential acids and when we hereinafter refer to the acids which furnish the cellulose-esterifying groups, we shall, for convenience, indicate by that term either said acids, or their anhydrids, or mixtures of them. For example, we may prepare a bath of 20 parts by weight of chloracetic anhydrid, 30 parts of chloracetic acid, 7 parts of stearic acid, 3 parts of acetic anhydrid and 0.1 part of magnesium perchlorate. In this are treated 4 parts by weight of cellulose for about 5 hours at 60° to 65° C. When a clear dope is formed, the cellulose ester is separated, as hereinabove described. This mixed ester is soluble in acetone, chloroform, and insoluble in benzene, being an acetostearate of cellulose.

While formic acid has certain chemical properties not found in the other fatty acids, our process can be carried out with it. For example, 20 parts by weight of formic acid (85% strength) and 40 parts of chloracetic anhydrid are warmed at 50° C. for one hour and cooled down to 30° C. Five parts by weight of cellulose are added to the mixture with stirring and the mixture kept at 35° to 40° C. for 96 hours. The mixture is poured into water, with agitation to precipitate the cellulose formate, which can be washed. It is completely soluble in acetone at room temperature, insoluble in chloroform and contains about 25.5% of the group HCO, corresponding closely to a diformate. While the reaction is preferably carried out for 96 hours, a clear dope may be formed as early as 24 hours; if the product be isolated at this stage, it is found to contain only 19% of the formyl group and to be insoluble in acetone.

Using the same reaction mixture and conditions in the preceding example, we can, after 48 hours of the reaction, add to the mixture 10 parts by weight of formic acid with 20 parts of chloracetic anhydrid and the reaction conducted 48 hours more. This gives, after precipitation and washing, a product somewhat higher than a diformate, which is soluble in acetone but not in chloroform and may contain 27.6% of the HCO group.

Moreover, the cellulose formate thus produced, may be further esterified by our process to obtain mixed esters. For example, 4½ parts by weight of an above described acetone-soluble cellulose formate are added to a mixture of 15 parts by weight of stearic acid, 20 parts of chloracetic anhydrid and .05 parts of magnesium perchlorate and the mass warmed and kept at 60° to 65° C. for about 72 hours. This may be precipitated in warm methyl alcohol. The mixed formostearate is soluble at room temperature in acetone, chloroform, or benzene, but insoluble in ligroin, ether, or carbon tetrachlorid.

- As an example of the use of red phosphorus and chlorine to catalyze the reaction, we note the following: Into 25 parts by weight of acetic acid and 35 parts of chloracetic anhydrid there are mixed 5 parts of cotton cellulose, and 0.2 parts of red phosphorus. This is treated with chlorine bubbling through it until the absorption of chlorine ceases. The mixture is then warmed between 60° to 68° C. until it becomes homogeneous. It is then poured into water and the product isolated by the usual known methods. This yields chloroform-soluble cellulose acetate, which may be hydrolyzed in the usual way.
- The halogen substituted anhydrids of the fatty acids are not the only substituted anhydrids of these acids which impel esterification without containing esterifying groups. Certain groups, such as the alkoxy group, behave like a halogen group in this respect when substituted in the same place in the fatty acid anhydrid. Take methoxyacetic anhydrid, for example. Mix 15 parts by weight of it with 10 parts of acetic acid and 0.10 parts of magnesium perchlorate and warm to 60° to 65° C. Into this are stirred 2 parts of cellulose, say tissue paper (cotton stock), and after 50 hours at the above temperature a clear dope results which, upon pouring into methyl alcohol, etc., yields a product soluble in chloroform and insoluble in acetone,—in other words, it yields fully acetylated cellulose which is, upon analysis, found to be substantially free from methoxy groups. Ethoxyacetic anhydrid and its higher alkyl homologues act like methoxyacetic anhydrid.
- It is a useful feature of our invention that it may be employed with commercial organic acids. For example, commercial stearic acid contains not only the pure stearic acid but also palmitic acid in considerable quantities. During the esterification, both of these acids enter from the mixture into the product and thus mixed esters may be prepared from commercial mixed acids. In the same way the saturated acids of cocoanut oil contain several acids of the fatty series, such as lauric and myristic, and all of these enter into the ester when such "a mixture" is utilized in our process. While we have also illustrated two mixed esters in which acyl groups of high and low molecular weight are used, namely, aceto-stearates and aceto-methoxybenzoates, it will be evident that any two or more of the organic acids in the group from which we make our selection, as specified above, may be used in forming mixed esters. This is extremely valuable, because, as indicated by the above examples, the solubilities of the products in different commercial organic solvents can be regulated by a proper selection of the esterifying acids and their proportions.
- While the chloracetic anhydrid is preferred, the di and tri-chloracetic anhydrids

are also useful. The mono, di, and tri bromoacetic anhydrids, or mixtures of them can be utilized. The mono, di, and tri chlor, and brom propionic and butyric anhydrids will operate, but they are too expensive to compete commercially. The corresponding iodine substituted acetic, propionic and butyric anhydrids are likewise expensive without proportional benefit. But whichever of the halogen substituted fatty acid anhydrids is employed, it is a characteristic of each of them that it will not contribute groups to the ester. Apparently the presence of the halogen in the molecule is the cause of this. Any substituted group in the anhydrid which prevents it from contributing groups to the ester can be used, such, for instance, as the methoxy group in methoxyacetic anhydrid. When properly purified, all of the esters produced by our process, contain no halogen atoms, except the ester of orthochlorbenzoic acid, which, of course, does not derive its halogen from the chloracetic anhydrid or chloracetic acid but only from the original orthochlorbenzoic acid.

The proportions in the above examples can be varied over a considerable range. The amount of chloracetic anhydrid can be greatly reduced to lessen the expense. It will be noted that our process is very economical in its use of the esterifying acids. For example, in the making of cellulose stearate from commercial stearic acid in the above table, the amount of stearic acid is only about 25% above that theoretically required. The yield, on the basis of the original cellulose is of the order of 250%.

It is a great advantage of our process that the esterification, especially of the mixed esters, can be carried out in one operation or by a single treatment in a single bath. If it be desired, for special reasons, to carry it out in a series of operations, our process can, of course, be used, the treatment being stopped at the different stages. Cellulose, which has been partially esterified, either by our method or by other methods, can be further or completely esterified by our method. For instance, as the cellulosic material, partially acetylated or nitrated cellulose may be substituted in equimolecular proportions for the cellulose in the above examples. Higher acid groups may be introduced in this way and aceto-laurates, aceto-palmitates and aceto-stearates or nitro-laurates, nitro-palmitates, and nitro-stearates produced. The acetylation can also be done by the process in our application Serial No. 122,028, filed July 12th, 1926, and higher acid groups, such as stearic, palmitic, or lauric, introduced by our present method.

It will be evident from the above description that we can produce a very large variety of esters of technical importance for the preparation of flexible, transparent photo-

graphic films, of filaments for making rayon, of lacquers, of artificial leather, of plastics and other fields in which cellulose esters have hitherto been employed. Many of the esters of the higher fatty acids and the aceto higher fatty acids have qualities which give them exceptional adaptability in this art. For example, they give flexible film or filaments without softeners or plastifiers; but the acetone-soluble or chloroform-soluble plasticizers, heretofore used with cellulose acetates, may be used with them. Triphenyl and tricresyl phosphates are good examples of the large number which can be used within the usual range of proportions. They can be mixed or laminated with cellulose nitrate or acetate by means of a common solvent. They can be backed with a cellulose acetate layer or with hygroscopic nitrocellulose coatings to prevent static, and these backings may have their electrical conductance improved by containing hygroscopic compounds.

Having thus described our invention, what we claim as new and desire to secure by Letters Patent is:

1. The process of making cellulose esters which comprises treating cellulosic material with an esterifying bath containing a halogen-substituted fatty acid anhydrid and an organic acid which contains an acyl group and which is selected from the group which consists of, first, the unsubstituted aliphatic monocarboxylic acids including the cycloparaffinic, second, the aromatic monocarboxylic acids, and, third, the aralkyl monocarboxylic acids.

2. The process of making cellulose esters which comprises treating cellulosic material with an esterifying bath containing as a source of esterifying groups at least one organic acid which contains an acyl group and which is selected from the group which consists of, first, the unsubstituted aliphatic monocarboxylic acids including the cycloparaffinic, second, the aromatic monocarboxylic acids and, third, the aralkyl monocarboxylic acids, and also containing as an impellent of esterification a halogen-substituted fatty acid anhydrid having less than ten carbon atoms.

3. The process of making cellulose esters which comprises treating cellulosic material with an esterifying bath containing as a source of esterifying groups at least one organic acid which contains an acyl group and which is selected from the group which consists of, first, the unsubstituted aliphatic monocarboxylic acids including the cycloparaffinic, second, the aromatic monocarboxylic acids, and also containing a halogen substituted acetic anhydrid to impel esterification and to form the corresponding halogen-substituted acetic acid as a solvent.

4. The process of making cellulose esters which comprises treating cellulosic material with a liquid esterifying mixture containing

an organic acid selected from the group which consists of, first, the unsubstituted aliphatic monocarboxylic acids including the cycloparaffinic, second, the aromatic monocarboxylic acids, and, third, the aralkyl monocarboxylic acids, and also containing chloracetic anhydrid.

5. The process of making cellulose esters which comprises treating cellulosic material with an esterifying bath containing an organic acid which contains an acyl group and which is selected from the group which consists of, first, the unsubstituted aliphatic monocarboxylic acids including the cycloparaffinic, second, the aromatic monocarboxylic acids, and, third, the aralkyl monocarboxylic acids, and a substituted fatty acid anhydrid which impels esterification of the cellulose by said first-named acid, but is prevented by the presence in it of the substituent group from contributing groups to the ester.

6. The process of making fatty acid esters of cellulose which comprises treating cellulosic material with an esterifying bath containing a halogen-substituted fatty acid anhydrid and an unsubstituted fatty acid.

7. The process of making stearyl-containing cellulose esters which comprises treating cellulosic material with an esterifying bath that includes a halogen-substituted fatty acid anhydrid and stearic acid.

8. The process of making cellulose esters which comprises treating cellulose with an esterifying bath containing an excess of organic acid over the amount required in the esterification reaction, said acid containing an acyl group and being selected from the group which consists of, first, the unsubstituted aliphatic monocarboxylic acids including the cycloparaffinic, second, the aromatic monocarboxylic acids, and, third, the aralkyl monocarboxylic acids, and also containing an excess of a halogen substituted fatty acid anhydrid over the amount required in the esterification reaction, said treatment being conducted at a temperature above the melting point of the bath but below the températures at which the cellulose and the ester are impaired.

9. The process of making fatty acid esters of cellulose which comprises treating cellulose with an esterifying bath containing an unsubstituted fatty acid, and a halogen-substituted fatty acid anhydrid containing less than ten carbon atoms.

10. The process of making fatty acid esters of cellulose which comprises treating cellulose with an esterifying bath containing chloracetic anhydrid, and an unsubstituted fatty acid, said treatment being conducted above the melting point of the bath but below 80° C.

11. The process of making stearyl-containing cellulose esters which comprises treating cellulose in an esterifying bath containing

chloracetic anhydrid, and stearic acid, the treatment being conducted above the melting point of the bath but below 80° C.

12. In the process for the manufacture of esters of cellulose with the higher homologues of acetic acid, the step which comprises treating cellulose with chloro acetic acid anhydride and a higher homologue of acetic acid with the addition of a catalyst.
- 10 13. In the process for the manufacture of esters of cellulose with the higher homologues of acetic acid, the step which comprises treating cellulose with chloro acetic acid anhydride and a monobasic fatty acid containing at least 3 and not more than 4 carbon atoms with the addition of a catalyst.
- 20 14. The process of making fatty acid esters of cellulose which comprises treating cellulose with an esterifying bath containing chloracetic anhydride, monochloracetic acid and a monobasic fatty acid containing at least 3 and not more than 4 carbon atoms.
- 25 15. The process of making a propionic ester of cellulose which comprises treating cellulose with an esterifying bath containing propionic acid, chloracetic anhydride and monochloracetic acid.
- 30 16. The process of making fatty acid esters of cellulose which comprises treating cellulose with an esterifying bath containing an unsubstituted fatty acid, chloracetic anhydride and monochloracetic acid.
- 35 17. The process of making fatty acid esters of cellulose which comprises treating cellulose with an esterifying bath containing a higher homologue of acetic acid, chloracetic anhydride and monochloracetic acid.
- 40 18. The process of making fatty acid esters of cellulose which comprises treating cellulosic material with an esterifying bath containing a substituted fatty acid anhydride which impels esterification of the cellulose, and a mono-basic fatty acid containing 3-4 carbon atoms.
- 45 19. The process of making fatty acid esters of cellulose which comprises treating cellulosic material with an esterifying bath containing chloracetic anhydride and a mono-basic fatty acid containing 3-4 carbon atoms.
- 50 20. The process of making a fatty acid ester of cellulose which comprises treating cellulosic material with an esterifying bath containing propionic acid and chloracetic anhydride.
- 55 21. The process of making a fatty acid ester of cellulose which comprises treating cellulosic material with an esterifying bath containing chloracetic anhydride, monochloracetic acid, and propionic acid.
- 60 22. Signed at Rochester, New York, this 23rd day of March, 1927.

HANS T. CLARKE.  
CARL J. MALM.